

- [54] **PROCESS FOR UPGRADING LUBRICATING OIL STOCK**
- [75] Inventors: **Robert F. Bridger, Hopewell; Costandi A. Audeh; El-Ahmadi I. Heiba, both of Princeton, all of N.J.**
- [73] Assignee: **Mobil Oil Corporation, New York, N.Y.**
- [21] Appl. No.: **694,003**
- [22] Filed: **Jun. 8, 1976**
- [51] Int. Cl.<sup>2</sup> ..... **C10G 29/04; C10G 29/10; C10G 29/16**
- [52] U.S. Cl. ..... **208/177; 208/288; 208/295; 208/296; 208/297; 208/299**
- [58] Field of Search ..... **208/208 R, 216, 243, 208/244, 247, 293, 288, 177, 295, 296, 299; 252/31**

[56] **References Cited**

**U.S. PATENT DOCUMENTS**

- |           |         |                |       |           |
|-----------|---------|----------------|-------|-----------|
| 1,795,278 | 3/1931  | Fischer        | ..... | 208/208 R |
| 2,854,399 | 9/1958  | Weller         | ..... | 208/293   |
| 2,985,586 | 5/1961  | Willson et al. | ..... | 208/216   |
| 3,904,511 | 9/1975  | Heiba et al.   | ..... | 208/288   |
| 3,917,566 | 11/1975 | Scott et al.   | ..... | 208/293   |

*Primary Examiner*—George Crasanakis

*Attorney, Agent, or Firm*—Charles A. Huggett; Raymond W. Barclay; Dennis P. Santini

[57] **ABSTRACT**

An improved process for preparing a stabilized lubricating oil resistant to oxidation and sludge formation upon exposure to a highly oxidative environment, such as when metals are present and an overbased component is present in the lubricating oil, is provided. In the present process wherein a lubricating oil stock to be upgraded is contacted with elemental sulfur in the presence of a catalyst material selected from the group consisting of alumina, aluminosilicate, a metal of Groups II-A, II-B, VI-B or VIII of the Periodic Table of Elements, an oxide of a metal of Groups II-A, II-B, VI-B or VIII, a sulfide of a metal of Groups II-A, II-B, VI-B or VIII, clay, silica, silica combined with an oxide of a metal of Groups II-A, III-A, IV-B or V-B, and combinations thereof, at relatively low temperatures of from about 150° to about 225° C, an improvement is provided which comprises conducting said contacting in a flow reactor or under conditions comparable to those existing in a flow reactor at a liquid hourly space velocity of from about 0.5 hr<sup>-1</sup> to about 20 hr<sup>-1</sup> whereby the amount of elemental sulfur required to provide a stabilized lubricating oil stock is significantly lower than when a batch reactor is utilized, thus facilitating subsequent removal of excess unreacted sulfur.

**6 Claims, No Drawings**

## PROCESS FOR UPGRADING LUBRICATING OIL STOCK

## BACKGROUND OF THE INVENTION

## 1. Field of the Invention

This invention relates to the production of improved lubricating oils. In particular, it relates to an improved method of preparation of stable lubricating oils which are highly resistant to oxidation and sludge formation when exposed to a highly oxidative environment.

## 2. Description of Prior Art

Hydrocarbon lubricating oils have been obtained by a variety of processes in which high boiling fractions are contacted with hydrogen in the presence of hydrogenation-dehydrogenation catalysts at elevated temperatures and pressures. In such processes there is a consumption of hydrogen. Lubricating oil fractions are separated from the resulting products. Such lubricating oil fractions differ from those obtained by fractional distillation of crude oils and the like, since they have such relatively high viscosity index values that solvent extraction treatments are generally not required to enhance their viscosity index values. Such lubricating oil fractions suffer from the shortcoming that they are 25 unstable when exposed to highly oxidative environments. When so exposed, sediment and lacquer formation occurs, thus lessening the commercial value of such lubricants.

Methods in the art directed to lessening such a shortcoming are exemplified by U.S. Pat. Nos. 3,436,334 and 3,530,061. They teach making a lubricating oil product fraction of hydrocracking resistant to deterioration upon exposure to light and air by contacting the lubricating oil fraction with a solid contacting agent having 35 hydrogenation-dehydrogenation properties under hydrogen pressure (U.S. Pat. No. 3,530,061); and making hydrocarbon lubricating oil resistant to such deterioration by contacting high boiling hydrocarbons with a hydrogenation-dehydrogenation catalyst and hydrogen (with hydrogen consumption), and thereafter dehydrogenating the resultant product on contact with a metal oxide or with metal and oxygen (U.S. Pat. No. 3,436,334). Both methods employ hydrogen atmosphere, high pressure and high temperature, i.e. 500° to 45 1000° F. No sulfur is employed in either patent method.

U.S. Pat. No. 3,904,511 teaches a batch operation process for stabilization of a lubricating oil stock which comprises contacting a high boiling hydrocarbon fraction lubricating oil stock with elemental sulfur in 50 amount of from 0.2 to 1.0 percent by weight of the oil stock in the presence of a catalyst.

The present invention is directed to an improved process and means for effecting substantial improvement in oxidative properties of lubricating oil by a low pressure, relatively low temperature partial dehydrogenation mechanism in the presence of a small amount of elemental sulfur, e.g. 0.025 to 0.2 weight percent, and a catalyst.

U.S. Pat. No. 2,604,438 teaches a "hydroforming" process for catalytic dehydrogenation of light (i.e. boiling at less than 600° F) hydrocarbon oils, presumably to increase aromatic content. The patent discloses the known fact that in processes of that nature, the presence of a small amount of sulfur in the feed has a beneficial 65 effect. It further states that when the oil to be "hydroformed" has no sulfur, i.e. no sulfur in the light hydrocarbon feed, then a small amount of sulfur, e.g. a

reducible sulfur compound, is added to the feed. The patent emphasizes that the invention disclosed therein "is only advantageous when the process is carried out at a temperature conducive to dehydrogenation, i.e. at a temperature of at least 825° F." Proclaimed in the patent is the fact that when lower temperatures are used, e.g. 150° to 225° C as in the present invention, "the described method offers no advantage."

The prior art practices of hydrofinishing and hydro-treating as a means of treatment of lubricating oil stocks (i.e. stocks boiling at temperatures over 600° F) leave behind the unstable oil fractions, i.e. hydroaromatic compounds, with labile hydrogen atoms such as, for example, fluorenes, benzofluorenes, acenaphthenes, tetralin, fused cycloalkylaromatics and naphthenes, which are quite unstable toward oxygen, particularly in the presence of metals in lubricating oil formulations containing overbased additives. These hydroaromatic compounds with labile hydrogen atoms are known to be present in small quantities in conventionally furfural refined stocks and can lead to oxidative instability of any lubricant containing them. Further, it is well known that the sensitivity of certain lubricating oils toward alkaline additives can cause oxidative degradation in applications where overbased additives are used, such as automotive and diesel lubricants. Also, metal sensitivity can be quite detrimental to the oxidative stability of lubricants or functional fluids in applications such as turbine circulating oils, steam turbine oils and hydraulic fluids. No method is known at present which so effectively and easily alleviates the above problems as the present invention.

## SUMMARY OF THE INVENTION

In accordance with the present invention there is provided an improved process and means for forming lubricating oils which are highly resistant to deterioration, e.g. oxidation and sludge formation, upon exposure to a highly oxidative environment.

The process of the present invention comprises contacting a lubricating oil stock, such as, for example, from a Midcontinental U.S.A. crude or an Arabian Light crude, in a flow reactor or under conditions comparable to those existing in a flow reactor with elemental sulfur in amount of from about 0.025 to about 0.2 percent by weight of the oil stock in the presence of a catalyst material selected from the group consisting of alumina, silica, an aluminosilicate, a metal of Groups II-A, II-B, VI-B or VIII of the Periodic Table of Elements, an oxide of a metal of Groups II-A, II-B, VI-B, or VIII, a sulfide of a metal of Groups II-A, II-B, VI-B or VIII, clay, silica combined with an oxide of a metal of Groups II-A, III-A, IV-B or V-B and combinations thereof.

The elemental sulfur for use herein may be provided for the treatment, if desired, by a sulfur precursor, such as, for example, H<sub>2</sub>S, an organosulfur compound, i.e. added or naturally occurring, or combinations thereof. Said naturally occurring organosulfur compound may be utilized if present in the lubricating oil stock in a quantity providing greater than about 0.125 weight percent sulfur. When such an organosulfur compound is the source of elemental sulfur herein, it can serve for generation of sulfur in situ. The catalyst materials for use in this invention serve to assist the extrusion of naturally occurring sulfur from the lubricating oil stock and, if sufficient organosulfur compounds are present therein, dehydrogenation is enhanced.

Non-limiting examples of sulfur precursors which may be utilized in the present process include  $H_2S$ ,  $RSH$ ,  $RS_xH$ ,  $HS_xH$ , and  $RS_xR$ , wherein  $R$  is a hydrocarbyl group and  $x$  is an integer of from 1 to 4 or more. Under actual operating conditions as herein set forth, these sulfur precursors, if used, can interact with the catalyst material for use herein to serve as a source of active sulfur in situ.

The treatment in accordance with the present invention may be followed, if desired, with various well known treatments such as thermal treatment or oxidation treatment in the presence of atmospheric oxygen and transition metal ions.

#### DESCRIPTION OF SPECIFIC EMBODIMENTS

The lubricating oil stocks which may be treated in accordance with the present invention may generally be any high boiling range materials boiling above about 600° F. Such lubricating oil stock materials include those obtained by fractionation, as by, for example, vacuum distillation, of crude oils identified by their source, i.e. Pennsylvania, Midcontinent, Gulf Coast, West Texas, Amal, Kuwait, Barco and Arabian. Said oil stock materials include one having a substantial part thereof of the fractionation product of the above crude oils mixed with other oil stocks.

The catalyst materials employed herein can include any type of catalyst which will bring about partial dehydrogenation and sulfur labilization (or sulfurization-desulfurization) when applied to the lubricating oil stock in the presence of elemental sulfur in very small quantity and at low operating temperature in an unpressured flow system. Such catalyst materials are known in the art for use in various other catalytic processes and include alumina, silica, silica combined with an oxide of a metal of Groups II-A, III-A, IV-B or V-B of the Periodic Table of Elements, such as, for example, silica-alumina, an aluminosilicate, a metal of Groups II-A, II-B, VI-B or VIII such as, for example, Mg, Ca, Zn, Cr, Mo, Fe, Co, Ni or Pt, an oxide of a metal of Groups II-A, II-B, VI-B or VIII such as  $CaO$ ,  $MgO$ ,  $Fe_2O_3$ ,  $MnO_2$ ,  $Cr_2O_3$  or  $ZnO$ , a sulfide of a metal of Groups II-A, II-B, VI-B or VIII such as, for example,  $Fe_2S$ ,  $Fe_2S_3$ ,  $FeS_2$ , (either marcasite or pyrite) or  $Fe_7S_8$  (pyrrhotite), certain clay and combinations thereof.

Non-limiting examples of the clays which may be useful as the catalyst material in the process of this invention include the montmorillonite and kaoline families, which families include the sub-bentonites and the kaolins commonly known as Dixie, McNamme, Georgia and Florida clays, or others in which the main mineral constituent is halloysite, kaoline, dickite, nacrite, attapulgite or anauxite. Such clays can be used in the raw state as mined or initially subjected to calcination, acid treatment or chemical modifications.

Non-limiting examples of siliceous materials useful as the catalyst in the present invention include silica and combinations thereof with oxides of metals of Groups II-A, III-A, IV-B and V-B, such as, for example, silica-alumina, silica-magnesia, silica-zirconia, silica-thoria, silica-beryllia, silica-titania, as well as ternary compositions of silica, such as, for example, silica-alumina-thoria and silica-alumina-zirconia.

Non-limiting examples of aluminosilicate materials which may be useful as the catalyst herein include the synthetic zeolites A, B, L, T, X, Y, ZK-4, ZK-5, ZSM-4, ZSM-5, ZSM-35, ZSM-38 and others, and the natural zeolites levynite, dachiartie, erionite, faujasite, analcite,

paulingite, noselite, phillipsite, chabazite, leucite, mordenite and others.

The catalyst loses some of its activity during use and, therefore, may be regenerated. The spent catalyst is contacted with a free oxygen-containing atmosphere at an elevated temperature sufficient to burn carbonaceous deposits from the catalyst. Conditions for regenerating the catalyst include a temperature between about 600° and 1,000° F, a pressure of from atmosphereic to about 500 pounds per square inch, a total gas flow rate of from about 1 to about 20 volumes per volume of catalyst per minute and an oxygen concentration of from about 0.1 percent to 100 percent. The oxygen can be diluted with steam, nitrogen or other inert gas.

10 The process of the present invention involves the partial incorporation of sulfur into the lubricating oil stock or the partial desulfurization of the oil stock in addition to the partial dehydrogenation of the oil stock. Said dehydrogenation is believed to involve oxidatively unstable fractions of said oil stock including, for example, the above mentioned hydroaromatics such as fluorenes, benzofluorenes, acenaphthenes, tetralin, fused cycloalkylaromatics, naphthenes and the like. The unstable hydrogen of said hydroaromatics is eliminated from the oil stock treated in accordance herewith as one or more of the forms  $H_2S$ ,  $RSH$ ,  $HS_xH$  and  $RS_xR$ , wherein  $R$  is a hydrocarbyl group and  $x$  is an integer ranging from 1 to about 4 or more.

15 The elemental sulfur employed in the process of the present invention may be in any of several allotropic forms such as  $S_6$ ,  $S_8$  or polymeric sulfur and may be used in very small amounts of from about 0.025 to about 0.2 percent by weight of oil stock, with a preferable range of from about 0.05 to about 0.15 percent by weight. It is readily observable that this invention differs from the well-known method of making sulfurized oil-extreme pressure agents in conditions of processing, the concept of improvement, the amount and type of sulfur incorporated and the chemical modification of the oil stock itself. In the present invention, small amounts of stable sulfur may be chemically incorporated into the oil molecules as labile hydrogen atoms are removed. On the other hand, in sulfurized oils used as extreme pressure agents, large quantities of sulfur, such as, for example, 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4096 4097 4098 4099 4100 4101 4102 4103 4104 4105 4106 4107 4108 4109 4110 4111 4112 4113 4114 4115 4116 4117 4118 4119 4120 4121 4122 4123 4124 4125 4126 4127 4128 4129 4130 4131 4132 4133 4134 4135 4136 4137 4138 4139 4140 4141 4142 4143 4144 4145 4146 4147 4148 4149 4150 4151 4152 4153 4154 4155 4156 4157 4158 4159 4160 4161 4162 4163 4164 4165 4166 4167 4168 4169 4170 4171 4172 4173 4174 4175 4176 4177 4178 4179 4180 4181 4182 4183 4184 4185 4186 4187 4188 4189 4190 4191 4192 4193 4194 4195 4196 4197 4198 4199 4199 4200 4201 4202 4203 4204 4205 4206 4207 4208 4209 4210 4211 4212 4213 4214 4215 4216 4217 4218 4219 4220 4221 4222 4223 4224 4225 4226 4227 4228 4229 4229 4230 4231 4232 4233 4234 4235 4236 4237 4238 4239 4239 4240 4241 4242 4243 4244 4245 4246 4247 4248 4249 4249 4250 4251 4252 4253 4254 4255 4256 4257 4258 4259 4259 4260 4261 4262 4263 4264 4265 4266 4267 4268 4269 4269 4270 4271 4272 4273 4274 4275 4276 4277 4278 4279 4279 4280 4281 4282 4283 4284 4285 4286 4287 4288 4289 4289 4290 4291 4292 4293 4294 4295 4296 4297 4298 4299 4299 4300 4301 4302 4303 4304 4305 4306 4307 4308 4309 4309 4310 4311 4312 4313 4314 4315 4316 4317 4318 4319 4319 4320 4321 4322 4323 4324 4325 4326 4327 4328 4329 4329 4330 4331 4332 4333 4334 4335 4336 4337 4338 4339 4339 4340 4341 4342 4343 4344 4345 4346 4347 4348 4349 4349 4350 4351 4352 4353 4354 4355 4356 4357 4358 4359 4359 4360 4361 4362 4363 4364 4365 4366 4367 4368 4369 4369 4370 4371 4372 4373 4374 4375 4376 4377 4378 4379 4379 4380 4381 4382 4383 4384 4385 4386 4387 4388 4389 4389 4390 4391 4392 4393 4394 4395 4396 4397 4398 4399 4399 4400 4401 4402 4403 4404 4405 4406 4407 4408 4409 4409 4410 4411 4412 4413 4414 4415 4416 4417 4418 4419 4419 4420 4421 4422 4423 4424 4425 4426 4427 4428 4429 4429 4430 4431 4432 4433 4434 4435 4436 4437 4438 4439 4439 4440 4441 4442 4443 4444 4445 4446 4447 4448 4449 4449 4450 4451 4452 4453 4454 4455 4456 4457 4458 4459 4459 4460 4461 4462 4463 4464 4465 4466 4467 4468 4469 4469 4470 4471 4472 4473 4474 4475 4476 4477 4478 4479 4479 4480 4481 4482 4483 4484 4485 4486 4487 4488 4489 4489 4490 4491 4492 4493 4494 4495 4496 4497 4498 4498 4499 4499 4500 4501 4502 4503 4504 4505 4506 4507 4508 4509 4509 4510 4511 4512 4513 4514 4515 4516 4517 4518 4519 4519 4520 4521 4522 4523 4524 4525 4526 4527 4528 4529 4529 4530 4531 4532 4533 4534 4535 4536 4537 4538 4539 4539 4540 4541 4542 4543 4544 4545 4546 4547 4548 4549 4549 4550 4551 4552 4553 4554 4555 4556 4557 4558 4559 4559 4560 4561 4562 4563 4564 4565 4566 4567 4568 4569 4569 4570 4571 4572 4573 4574 4575 4576 4577 4578 4579 4579 4580 4581 4582 4583 4584 4585 4586 4587 4588 4589 4589 4590 4591 4592 4593 4594 4595 4596 4597 4598 4598 4599 4599 4600 4601 4602 4603 4604 4605 4606 4607 4608 4609 4609 4610 4611 4612 4613 4614 4615 4616 4617 4618 4619 4619 4620 4621 4622 4623 4624 4625 4626 4627 4628 4629 4629 4630 4631 4632 4633 4634 4635 4636 4637 4638 4639 4639 4640 4641 4642 4643 4644 4645 4646 4647 4648 4649 4649 4650 4651 4652 4653 4654 4655 4656 4657 4658 4659 4659 4660 4661 4662 4663 4664 4665 4666 4667 4668 4669 4669 4670 4671 4672 4673 4674 4675 4676 4677 4678 4679 4679 4680 4681 4682 4683 4684 4685 4686 4687 4688 4689 4689 4690 4691 4692 4693 4694 4695 4696 4697 4698 4698 4699 4699 4700 4701 4702 4703 4704 4705 4706 4707 4708 4709 4709 4710 4711 4712 4713 4714 4715 4716 4717 4718 4719 4719 4720 4721 4722 4723 4724 4725 4726 4727 4728 4729 4729 4730 4731 4732 4733 4734 4735 4736 4737 4738 4739 4739 4740 4741 4742 4743 4744 4745 4746 4747 4748 4749 4749 4750 4751 4752 4753 4754 4755 4756 4757 4758 4759 4759 4760 4761 4762 4763 4764 4765 4766 4767 4768 4769 4769 4770 4771 4772 4773 4774 4775 4776 4777 4778 4779 4779 4780 4781 4782 4783 4784 4785 4786 4787 4788 4789 4789 4790 4791 4792 4793 4794 4795 4796 4797 4798 4798 4799 4799 4800 4801 4802 4803 4804 4805 4806 4807 4808 4809 4809 4810 4811 4812 4813 4814 4815 4816 4817 4818 4819 4819 4820 4821 4822 4823 4824 4825 4826 4827 4828 4829 4829 4830 4831 4832 4833 4834 4835 4836 4837 4838 4839 4839 4840 4841 4842 4843 4844 4845 4846 4847 4848 4849 4849 4850 4851 4852 4853 4854 4855 4856 4857 4858 4859 4859 4860 4861 4862 4863 4864 4865 4866 4867 4868 4869 4869 4870 4871 4872 4873 4874 4875 4876 4877 4878 4878 4879 4880 4881 4882 4883 4884 4885 4886 4887 4888 4889 4889 4890 4891 4892 4893 4894 4895 4896 4897 4898 4898 4899 4899 4900 4901 4902 4903 4904 4905 4906 4907 4908 4909 4909 4910 4911 4912 4913 4914 4915 4916 4917 4918 4919 4919 4920 4921 4922 4923 4924 4925 4926 4927 4928 4929 4929 4930 4931 4932 4933 4934 4935 4936 4937 4938 4939 4939 4940 4941 4942 4943 4944 4945 4946 4947 4948 4949 4949 4950 4951 4952 4953 4954 4955 4956 4957 4958 4959 4959 4960 4961 4962 4963 4964 4965 4966 4967 4968 4969 4969 4970 4971 4972 4973 4974 4975 4976 4977 4978 4978 4979 4980 4981 4982 4983 4984 4985 4986 4987 4988 4989 4989 4990 4991 4992 4993 4994 4995 4996 4997 4998 4998 4999 4999 5000 5001 5002 5003 5004 5005 5006 5007 5008 5009 5009 5010 5011 5012 5013 5014 5015 5016 5017 5018 5019 5019 5020 5021 5022 5023 5024 5025 5026 5027 5028 5029 5029 5030 5031 5032 5033 5034 5035 5036 5037 5038 5039 5039 5040 5041 5042 5043 5044 5045 5046 5047 5048 5049 5049 5050 5051 5052 5053 5054 5055 5056 5057 5058 5059 5059 5060 5061 5062 5063 5064 5065 5066 5067 5068 5069 5069 5070 5071 5072 5073 5074 5075 5076 5077 5078 5079 5079 5080 5081 5082 5083 5084 5085 5086 5087 5088 5089 5089 5090 5091 5092 5093 5094 5095 5096 5097 5098 5098 5099 5099

degree of improvement or upgrading product quality of the lubricating oil stock treated without loss in yield. Aside from specific small amounts of sulfur, the reaction temperature must be within the range of from about 150° to about 225° C, preferably from about 160° to 5 about 180° C. The reaction pressure may be from about 0 psig to about 500 psig, preferably from about 0 psig to about 200 psig. Liquid hourly space velocity (LHSV) must be maintained within the range of from about 0.5 to about 20 hr<sup>-1</sup> (vol. oil/vol. catalyst), preferably from about 1 to about 10 hr<sup>-1</sup> and more preferably from about 1 to about 5 hr<sup>-1</sup>.

By using the improved flow process of the present invention, a smaller concentration of elemental sulfur is required than if a batch process, e.g. U.S. Pat. No. 15 3,904,511, is used. When the batch process is used, there is needed from about 0.2 to about 1.0 percent by weight of the oil stock being treated of elemental sulfur. When the present flow process is used, i.e. a flow reactor or 20 conditions comparable to those existing in a flow reactor, only from about 0.025 to about 0.2 percent by weight of the oil stock being treated of elemental sulfur is needed. Economic and processing benefits from the 25 present process when compared to those of the prior art are readily noted. One such benefit is, of course, that removal of excess unreacted sulfur from the oil stock treated hereby is greatly facilitated. Further, corrosion problems inherent in the use of larger amounts of sulfur are solved.

In order to more fully illustrate the process of the 30 present invention, the following specific examples, which in no sense limit the invention, are presented. The basic test procedure employed in evaluation of product yield from the present process is described by Dornte in *Industrial and Engineering Chemistry*, 28, 35 26-30, 1936 modified as below indicated.

It is interesting to note that performance of a lubricating oil in the below described test method is indicative of that oil's performance in the field. The test is conducted in an air circulation apparatus of the type described by Dornte. A tube containing 30 grams of lubricating oil (with or without additive) is placed in a heater thermostatted at 162° C. Air is circulated through the oil sample at a rate of 5 liters per hour. Metal surfaces 40 are provided for oil contact to act as oxidation accelerators. The metal surfaces employed include: iron wire, analytical grade, Washburn and Moen No. 15 gage, wound into a coil approximately  $\frac{1}{8}$  inch O.D. and 2 $\frac{1}{2}$  inches long to give a surface area of approximately 15.3 square inches; copper wire, electrolytic, B and S gage No. 18, 6.2 inches long; and a lead (tin-free) square 0.25 inch  $\times$  0.25 inch cut from 1/16 inch thick sheet. 45

Another test method used herein is the standard Rotary Bomb Oxidation Test (RBOT) designated ASTM D2272. Each sample tested in the RBOT test was 55 blended with a standard commercial additive package prior to testing.

The lubricating oil stock used in the following examples was conventionally refined by distillation, followed by furfural extraction and methyl ethyl ketone dewaxing. It is identified in Table 1 according to source, physical properties and furfural extraction conditions.

TABLE 1

| CRUDE SOURCE AND NOMINAL VISCOSITY<br>OF LUBRICATING OIL STOCK USED HEREIN |               |
|----------------------------------------------------------------------------|---------------|
| 150 S.U.S.                                                                 | Arabian Light |

Furfural Dosage,

TABLE 1-continued

| CRUDE SOURCE AND NOMINAL VISCOSITY<br>OF LUBRICATING OIL STOCK USED HEREIN |                 |
|----------------------------------------------------------------------------|-----------------|
| 150 S.U.S.                                                                 | Arabian Light   |
| % volume                                                                   | 180             |
| Tower Temp., °F, Top                                                       | 185             |
| Tower Temp., °F, Bottom                                                    | 140             |
| Gravity, °API                                                              | 30.9            |
| Pour Pt., °F                                                               | 0               |
| Flash Pt., °F                                                              | 410             |
| Sulfur, % wt.                                                              | 0.63            |
| Nitrogen, % wt.                                                            | 0.0029          |
| Aniline Point, °F                                                          | 210             |
| Viscosity, S.U.S. at<br>100° F                                             | 152             |
| Viscosity Index                                                            | 103             |
| ASTM Color                                                                 | 1 $\frac{1}{2}$ |

## EXAMPLE 1

A 50 gram quantity of the above oil stock, without treatment in accordance with the present invention, was subjected to the RBOT test and a 30 gram quantity of the untreated oil was subjected to the above-described Dornte test. The results of the tests are recorded in Table 2 for comparison purposes with tests conducted on the same oil stock treated by the present process (Examples 2-5).

## EXAMPLE 2

A 450 gram quantity of the above oil stock was mixed with 0.2 weight percent of elemental sulfur (based on weight of oil) and allowed to flow through a reactor containing 10 grams of 1/16-inch extrudate zeolite X (i.e. NaX). The reaction temperature was maintained at 175° C, the reaction pressure was maintained at 25 psig and the LHSV was 1 hr<sup>-1</sup>. The oil was then cooled to room temperature and residual corrosive sulfur was removed by stirring the oil with finely divided sodium hydroxide (50 grams) for 16 hours. After removal of the sodium hydroxide by filtration, the oil was tested in the RBOT and Dornte tests, and shown to have improved oxidation properties, as demonstrated in Table 2.

The flow reactor used was a 15 ml. downflow reactor.

## EXAMPLE 3

A 450 gram quantity of the above oil stock was mixed with 0.1 weight percent of elemental sulfur (based on weight of oil) and allowed to flow through the reactor and under the reaction conditions of Example 2. The oil was then washed with sodium hydroxide, filtered and tested as in Example 2. The results, showing improved oxidation properties, are recorded in Table 2.

## EXAMPLE 4

A 450 gram quantity of the above oil stock was mixed with 0.05 weight percent of elemental sulfur (based on weight of oil) and allowed to flow through the reactor and under the reaction conditions of Example 2. The oil was then washed with sodium hydroxide, filtered and tested as in Example 2. The results, showing improved oxidation properties, are recorded in Table 2.

## EXAMPLE 5

A 450 gram quantity of the above oil stock was mixed with 0.025 weight percent of elemental sulfur (based on weight of oil) and allowed to flow through the reactor and under the reaction conditions of Example 2. The oil was then washed with sodium hydroxide, filtered and

tested as in Example 2. The results, showing improved oxidation properties, are recorded in Table 2.

#### EXAMPLE 6

In order to demonstrate the beneficial effect of the present flow process over that of the art whereby the sulfur contacting is conducted in a stirred batch reactor (i.e. as in U.S. Pat. No. 3,904,511), a 450 gram quantity of the above oil stock was thermostatted under nitrogen at 175° C in the presence of 10 grams of the zeolite catalyst used in above Examples 2-5. Elemental sulfur (2.25 grams) was added and the oil was stirred at 175° C for 1 hour while hydrogen sulfide was evolved. The oil was cooled to room temperature and residual corrosive sulfur was removed by stirring the oil with finely divided sodium hydroxide as in Examples 2-5. The product was filtered and tested as in Examples 2-5 and the results of the tests are recorded in Table 2.

#### EXAMPLE 7

Further in demonstration of the beneficial effect of the present flow process over that of the art whereby the sulfur contacting is conducted in a stirred batch reactor (i.e. as in U.S. Pat. No. 3,904,511), a 450 gram quantity of the above oil stock is thermostatted under nitrogen at 175° C in the presence of 10 grams of the zeolite catalyst used in above Examples 2-5. Elemental sulfur (0.45 grams) is added and the oil is stirred at 175° C for 1 hour while hydrogen sulfide is evolved. The oil is cooled to room temperature and residual corrosive sulfur is removed by stirring the oil with finely divided sodium hydroxide as in Examples 2-5. The product is filtered and tested as in Examples 2-5 and the results of the tests are recorded in Table 2.

TABLE 2

| Example      | Oxidation Test Results of Examples 1-7 |                |
|--------------|----------------------------------------|----------------|
|              | RBOT, minutes                          | Dornte, hours* |
| 1            | 268                                    | 43.3           |
| 2            | 360                                    | 86.3           |
| 2 (repeated) | —                                      | 90.9           |
| 3            | 395                                    | 59.5           |
| 4            | 400                                    | 79.0           |
| 5            | 420                                    | 63.4           |
| 6            | 343                                    | 65.2           |
| 6 (repeated) | 345                                    | 77.3           |
| 7            | 300                                    | 45.1           |

\*Time required for absorption of 1 mole O<sub>2</sub> per kg oil at 162° C with Fe, Cu and Pb present.

#### EXAMPLE 8

In the flow reactor of Example 2 containing 15 ml. of 1/16-inch extrudate zeolite X, i.e. NaX, and with the temperature maintained at 175° C, the pressure at 25 psig and the LHSV at 1 hr<sup>-1</sup>, the above oil stock was contacted with elemental sulfur in four different concentrations varied with time on stream to examine degree of dehydrogenation of the oil stock. The initial contacting was at 0.2 weight percent elemental sulfur (based on weight of oil). At 113 hours on stream, the contacting was changed to 0.1 weight percent elemental sulfur. At 141 hours on stream, the contacting was changed to 0.05 weight percent elemental sulfur and at 168 hours, to 0.025 weight percent elemental sulfur. Results indicated that stable oil can be produced at much lower degrees of reaction than previously suspected since good oxidation stabilities (see Table 2) were obtained in the range of only 0.028 to 0.17 mole percent of oil reacted (see results of Example 8 in Table 3).

TABLE 3

| Dehydrogenation of Lubricating Oil Stock in Example 8 |       |                      |               |                                      |
|-------------------------------------------------------|-------|----------------------|---------------|--------------------------------------|
| Hours on Stream                                       | % S*  | % H <sub>2</sub> S** | % S Converted | Oil Stock Converted, mole percent*** |
| 0 - 113                                               | 0.2   | 0.0145               | 7.25          | 0.17                                 |
| 113 - 141                                             | 0.1   | 0.0054               | 5.40          | 0.063                                |
| 141 - 168                                             | 0.05  | 0.0039               | 7.80          | 0.046                                |
| 168 - 193                                             | 0.025 | 0.0024               | 9.60          | 0.028                                |

\*Weight percent of elemental sulfur contacted with the oil stock in the flow reactor.

\*\*Weight percent of H<sub>2</sub>S formed in the oil stock.

\*\*\*Assuming a molecular weight of oil stock at 400, this value is 100 × moles H<sub>2</sub>S/mole of oil.

#### EXAMPLES 9-12

These examples were conducted in the flow reactor of Example 2 containing 10 grams of 1/16-inch extrudate zeolite X (i.e. NaX). The weight percent of elemental sulfur used (basis of 450 grams oil stock identified above) and the reaction conditions were varied, as indicated in Table 4. The treated oil was washed, filtered and tested (RBOT) as in Example 2 and the results of the tests appear in Table 4.

#### EXAMPLE 13

A 450 gram quantity of the above oil stock is mixed with 0.2 weight percent of elemental sulfur (based on weight of oil) and allowed to flow through the reactor of Example 2 containing 10 grams of 1/16-inch extrudate mordenite zeolite. The oil is then washed, filtered and tested (RBOT) as in Example 2. The reaction conditions and test results are recorded in Table 4.

#### EXAMPLE 14

A 450 gram quantity of the above oil stock was mixed with 0.1 weight percent of elemental sulfur and allowed to flow through the reactor of Example 2 containing 10 grams of 8-12 mesh rare earth exchanged zeolite Y. The oil was then washed, filtered and tested (RBOT) as in Example 2. The reaction conditions and test results are recorded in Table 4.

#### EXAMPLE 15

A 450 gram quantity of the above oil stock is mixed with 0.2 weight percent of elemental sulfur and allowed to flow through the reactor of Example 2 containing 10 grams of 8-12 mesh silica. The oil is then washed, filtered and tested (RBOT) as in Example 2. The reaction conditions and test results are recorded in Table 4.

#### EXAMPLE 16

A 450 gram quantity of the above oil stock is mixed with 0.2 weight percent of elemental sulfur and allowed to flow through the reactor of Example 2 containing 10 grams of 40 mesh silica-alumina. The oil is then washed, filtered and tested (RBOT) as in Example 2. The reaction conditions and test results are recorded in Table 4.

TABLE 4

| Ex. | Reaction Conditions and Oxidation Test Results of Examples 9-16 |          |                |                        |               |
|-----|-----------------------------------------------------------------|----------|----------------|------------------------|---------------|
|     | S* wt. %                                                        | Temp. °C | Pressure psig. | LHSV, hr <sup>-1</sup> | RBOT, minutes |
| 9   | 0.1                                                             | 160      | 25             | 1                      | 360           |
| 10  | 0.05                                                            | 175      | 25             | 5                      | 400           |
| 11  | 0.025                                                           | 175      | 50             | 10                     | 420           |
| 12  | 0.15                                                            | 180      | 25             | 7.2                    | 350           |
| 13  | 0.2                                                             | 175      | 25             | 0.5                    | 345           |
| 14  | 0.1                                                             | 175      | 25             | 1                      | 347           |
| 15  | 0.2                                                             | 225      | 500            | 1                      | 330           |

TABLE 4-continued

| Reaction Conditions and Oxidation Test Results<br>of Examples 9-16 |             |             |                   |                           |
|--------------------------------------------------------------------|-------------|-------------|-------------------|---------------------------|
| Ex.                                                                | S*<br>wt. % | Temp.<br>°C | Pressure<br>psig. | LHSV,<br>hr <sup>-1</sup> |
| 16                                                                 | 0.2         | 150         | 75                | 2                         |
|                                                                    |             |             |                   | 335                       |

\*Weight percent of elemental sulfur mixed with the oil stock which is allowed to flow through the reactor of Example 2.

In contrast with prior art results in a stirred batch reactor, it is now found that better improvement of a lubricating oil stock in oxidation stability is obtained at both lower sulfur levels and lower degrees of dehydrogenation. In a stirred batch reactor, optimum sulfur concentration is about 0.5 weight percent. In the present process, optimum sulfur concentration is less than 0.2 weight percent.

At the low sulfur concentrations of the present invention, catalyst aging does not appear significant. Further, operating at lower sulfur levels will simplify removal of corrosive sulfur materials from the oil by post-treatment.

Having thus given a general description of the process and means of this invention and provided by way of examples specific embodiments thereof, it is to be understood that no undue restrictions are to be imposed by reason thereof, and minor modifications may be made thereto without departing from the scope thereof.

What is claimed is:

1. In a process for preparing a stabilized lubricating oil resistant to oxidation and sludge formation upon exposure to a highly oxidative environment which comprises contacting a hydrocarbon fraction lubricating oil stock boiling above about 600° F with added elemental sulfur, said contacting in the presence of a catalyst material selected from the group consisting of alumina,

30  
35

aluminosilicate, a metal of Groups II-A, II-B, VI-B or VIII of the Periodic Table of Elements, an oxide of a metal of Groups II-A, II-B, VI-B or VIII, a sulfide of a metal of Groups II-A, II-B, VI-B or VIII, clay, silica, silica combined with an oxide of a metal of Groups II-A, III-A, IV-B or V-B, and combinations thereof at a reaction temperature of from about 150° to about 225° C and a reaction pressure of from about 0 psig to about 500 psig, the improvement which comprises conducting said contacting in a flow reactor at a liquid hourly space velocity of from about 0.5 hr<sup>-1</sup> to about 20 hr<sup>-1</sup> wherein said elemental sulfur is added in an amount of from about 0.025 to about 0.2 percent by weight of said oil stock.

10  
15  
20  
25  
30  
35

2. The process of claim 1 wherein said elemental sulfur is added in amount of from about 0.05 to about 0.15 percent by weight of said oil stock, said reaction temperature is from about 160° to about 180° C, said reaction pressure is from about 0 psig to about 200 psig, and said liquid hourly space velocity is from about 1 hr<sup>-1</sup> to about 10 hr<sup>-1</sup>.

3. The process of claim 2 wherein said liquid hourly space velocity is from about 1 hr<sup>-1</sup> to about 5 hr<sup>-1</sup>.

4. The process of claim 1 wherein said contacting is in the presence of said catalyst material in conjunction with a secondary agent selected from the group consisting of bases.

5. The process of claim 4 wherein said base is sodium hydroxide.

6. The process of claim 1 wherein said oil stock comprises at least a substantial part of one obtained by fractionation of a crude oil identified as Pennsylvania, Mid-continent, Gulf Coast, West Texas, Amal, Kuwait, Barco or Arabian.

\* \* \* \* \*